

Oct. 27, 1931.

R. K. MILLER

1,829,417

REFRIGERATING APPARATUS

Filed Nov. 30, 1927



Fig. 2

Ralph K. Miller <sup>Inventor</sup>

By Spencer Hardman & Felt

Attorney

## UNITED STATES PATENT OFFICE

RALPH K. MILLER, OF DAYTON, OHIO, ASSIGNOR, BY MESNE ASSIGNMENTS, TO FRIGID-AIRE CORPORATION, A CORPORATION OF DELAWARE

## REFRIGERATING APPARATUS

Application filed November 30, 1927. Serial No. 236,717.

This invention relates to refrigerating apparatus and particularly to a novel method of lubricating such apparatus.

One of the objects of the invention is to provide positive and regular circulation of lubricant in refrigerating apparatus. More specifically it is an object of the invention to return lubricant from the evaporating or expander to the compressor of a refrigerating system.

Further objects and advantages of the present invention will be apparent from the following description, reference being had to the accompanying drawings, wherein a preferred form of the present invention is clearly shown.

In the drawings:

Fig. 1 is a conventional or diagrammatic representation of a refrigerating system in which my invention is embodied, and

Fig. 2 is a vertical longitudinal section thru a portion of the evaporator of such system.

Fig. 1 shows a compressor-condenser-expander type of refrigerating apparatus having an evaporator 10 and a condensing element including a compressor 11, a condenser 12, and a receiver, or liquid refrigerant tank 13. Refrigerant vapor is withdrawn from the evaporator thru the vapor or low pressure conduit 14 and is liquefied in the condenser 12 and returned to the evaporator thru the liquid or high pressure conduit 15. The compressor is operated by a motor 17 controlled by an automatic switch 18 which may be actuated in response to the refrigerating demand, for example by a pressure responsive device 19 connected to the low pressure conduit 14.

Referring to Fig. 2, the evaporator comprises a header 20 forming a reservoir for liquid refrigerant, and a number of tubes or ducts 21 depending from the header for circulating refrigerant. The liquid refrigerant is indicated by 22 and is kept at a constant level 23 by a valve 24 actuated by a float 25. The liquid refrigerant is supplied by a

connection 15' and the vapor is withdrawn thru a tube 14' connected to the vapor conduit 14.

All of the apparatus above described is well known in the art and its particular form and arrangement is immaterial to the present invention. It has been customary to lubricate the compressor of such systems by placing a quantity of oil in the crank case and depending upon the splashing of the rotating parts to distribute the oil thruout the compressor. Some of the oil is dissolved in the refrigerant, and some of the oil is mechanically pumped by the compressor to the condenser and receiver and eventually to the evaporator. The refrigerant boils off in the evaporator, leaving the oil, which collects in a layer from  $\frac{1}{2}$  inch to  $1\frac{3}{4}$  inches thick on top of the refrigerant.

A great deal of trouble has been experienced in the past because this oil could not be effectively removed from the evaporator. Not only does the collection of oil in the evaporator exhaust the supply of lubricant in the compressor, but it also hinders evaporation of the refrigerant, causing the pressure and consequently the temperature of the refrigerant to increase. Various arrangements have been attempted for periodically or regularly extracting this oil from the evaporator and returning it to the compressor. One of those proposed and widely in use is the evaporator exhaust connection 14' shown in Fig. 2. This is a tube projecting into the evaporator and having its open end 25 above the level of the oil layer. One or more drain openings 26 are formed in the side of the tube below the level of the opening 25 and also below the estimated level of the oil but above the estimated level of the liquid refrigerant. The theory of this arrangement is that the refrigerant vapor will be withdrawn from the top of the header thru the opening 25 by the suction of the compressor and that whenever the oil level 90

reaches the opening 26, oil will drain out of the evaporator. However, this arrangement has proved unsatisfactory and unreliable in service, and as far as I am aware, no plan for removing oil has been completely successful. It is well known that evaporators of this character may collect oil until the compressor is completely dry, and that while oil may be returned to the compressor at intervals, the return is extremely irregular and the apparatus will frequently operate as much as sixty days without returning any oil whatever to the compressor.

I have discovered that the oils heretofore used for refrigerating apparatus lie on top of the refrigerant in a thick layer which is quite solid and is free from bubbles except as it is disturbed by the boiling of the refrigerant beneath it and the escape of the refrigerant thru it. When boiling of the refrigerant ceases, the few bubbles formed by the ebullition rapidly disappear. I have also discovered that there are certain oils, not heretofore used for refrigerating apparatus, which when used in such an evaporator form a deep but light and fluffy layer of sustained bubbles. That is, the boiling of the refrigerant causes the oil to foam and form a layer of bubbles which may even reach the top of the evaporator. When boiling of the refrigerant ceases, these bubbles do not immediately disappear but retain their form for a considerable period. The relative behavior of the two oils mentioned above may be roughly compared to boiling pure water and boiling soap solution respectively.

This discovery has enabled me to devise a new method of lubricating refrigerating apparatus. In accordance with this method I use as lubricant in the apparatus one of the last-mentioned oils, which I term "foaming oil". By this term I mean any oil which, when mixed with refrigerant, is capable of forming sustained bubbles or foam in appreciable quantities. In so doing I prefer to calibrate the float 25 so that the refrigerant level is considerably below the level of the outlet, as indicated in Fig. 2. That is, I leave an appreciable space between the surface of the liquid, whether oil or refrigerant, and the outlet, so that oil and vapor may be easily withdrawn without danger of splashing liquid refrigerant into the outlet. When the refrigerant is boiling, the oil (because of its foaming characteristics) forms bubbles or bodies of refrigerant vapor totally enclosed by films of oil. The suction produced by the compressor withdraws these bubbles thru the exhaust tube 14' and it will be evident that each time a bubble is drawn into the outlet, a certain quantity of refrigerant vapor and a certain quantity of oil is positively returned to the compressor. Since the oil foams up over the end of the exhaust conduit, refrigerant vapor can not be with-

drawn without removing this definite quantity of oil, consequently a positive and regular circulation of oil is effected.

I have also discovered that while the oil previously used will form a very thick layer on top of the refrigerant, sometimes as much as  $1\frac{3}{4}$  inches, these foaming oils do not form such a thick layer. The maximum thickness of the foaming oil layer which I have observed is about  $\frac{1}{2}$  inch. This characteristic materially improves the operation of the evaporator, because the boiling temperature of the refrigerant is not increased materially by this thin layer of oil.

The oils which I have found particularly suitable are certain paraffin base oils from the Pennsylvania district, and it is essential that these oils remain in a homogeneous liquid state at all temperatures encountered in the refrigerating apparatus. By "homogeneous liquid state" I mean that the oil must remain sufficiently fluid to flow readily and must remain free from suspended solid bodies such as crystals or particles of paraffin at the temperatures encountered in refrigerating practice, for example at temperatures as low as  $15^{\circ}$  F. Attempts have previously been made to use paraffin base oils in refrigerating apparatus but it was found that solid paraffin would separate out from such oils within the ordinary temperature range of refrigerating apparatus. It was also found that at the temperatures produced by ordinary refrigerating apparatus such oils would congeal. Either the separation of paraffin or the congelation rendered the oil unfit for use in refrigerating apparatus, and for these reasons paraffin base oils have not been used.

Ordinary paraffin oils have a pour point in the neighborhood of  $30^{\circ}$  F., whereas it has been usual, in ordinary domestic mechanical refrigerating apparatus, to specify oil having a pour point of  $-30^{\circ}$  F. By this is meant that the oil will pour readily from a container at this temperature. I have discovered that in the case of foaming oils, oils of a considerably higher pour point may be used successfully. For example one of the foaming oils which I have used successfully has a pour point of  $5^{\circ}$  F. When this oil is mixed with a refrigerant, such as sulphur dioxide, two liquid phases are formed which are generally called the sulphur dioxide phase and the oil phase. The sulphur dioxide phase appears to be and acts very much like sulphur dioxide, but is really a solution of a small proportion of oil in sulphur dioxide. The oil phase appears and acts very much like oil but this is in fact a solution of a small proportion of sulphur dioxide in oil. In the particular case under discussion the oil phase remains in a homogeneous liquid state and has a pour point as low as  $-27^{\circ}$  F. The reduction of the pour point from  $5^{\circ}$  to  $-27^{\circ}$

may possibly be due to the dissolving of the sulphur dioxide in the oil.

I have found that a paraffin base oil made by the Kendall Refining Company, Bradford, Pennsylvania, and having the following physical characteristics is suitable for my purpose:

|                                                   |          |
|---------------------------------------------------|----------|
| Specific gravity at 60° F.                        | .8665    |
| 10 Viscosity (Saybolt) at 100° F.                 | 94 sec.  |
| Viscosity (Saybolt) at 21° F.                     | 973 sec. |
| Flash point                                       | 360° F.  |
| Fire point                                        | 425° F.  |
| 15 Cold H <sub>2</sub> SO <sub>4</sub> absorption | 2.48%    |
| Pour point                                        | 5° F.    |

While I have described my invention as ascribed to an evaporator of the flooded type it will be understood that the method of lubrication is equally applicable to other kinds of evaporators such as the dry expansion type. Also while I have described my method of lubrication as involving a paraffin base oil, I wish it to be understood that the invention is not limited to this type of oil, any oil having the above described foaming characteristics being suitable. For example, I may add materials to asphalt base oils which will impart a foaming characteristic to such oils without detracting from their other characteristics which render them suitable for refrigeration.

What is claimed is as follows:

1. The method of operating refrigerating apparatus which consists in circulating through the apparatus a volatile refrigerant and oil capable of forming sustained bubbles in the presence of the refrigerant.

2. The method of removing both refrigerant and lubricant from a refrigerating evaporator which consists in evaporating the liquid refrigerant, forming sustained bubbles of refrigerant vapor and liquid lubricant, and removing the bubbles from the evaporator.

45 3. The method of circulating refrigerant and lubricant in a refrigerating system which comprises introducing liquid refrigerant and liquid lubricant into an evaporator, evaporating the refrigerant, forming sustained bubbles of refrigerant vapor and lubricant and removing the bubbles from the evaporator.

4. The method of circulating refrigerant and lubricant in a refrigerating system which comprises introducing into an evaporator liquid refrigerant and oil capable of forming sustained bubbles in the presence of the refrigerant, evaporating the refrigerant, forming sustained bubbles of refrigerant vapor and oil, and removing the bubbles from the evaporator.

55 5. Refrigerating apparatus comprising in combination a closed system including an evaporating element and a condensing element connected thereto, the system contain-

ing a volatile refrigerant and oil capable of forming sustained bubbles in the presence of the refrigerant.

6. The method of operating refrigerating apparatus which consists in circulating through the apparatus sulphur dioxide and oil capable of forming sustained bubbles in the presence of the refrigerant.

7. The method of removing sulphur dioxide and liquid lubricant from a refrigerating evaporator which consists in evaporating the sulphur dioxide, forming sustained bubbles of sulphur dioxide vapor and liquid lubricant, and removing the bubbles from the evaporator.

8. The method of circulating refrigerant and lubricant in a refrigerating system which comprises introducing liquid sulphur dioxide and liquid lubricant into an evaporator, evaporating the sulphur dioxide, forming sustained bubbles of sulphur dioxide and the lubricant and removing the bubbles from the evaporator.

9. The method of circulating refrigerant and lubricant in a refrigerating system which comprises introducing into an evaporator sulphur dioxide and oil capable of forming sustained bubbles in the presence of sulphur dioxide, evaporating the sulphur dioxide, forming sustained bubbles of sulphur dioxide vapor and the foaming oil, and removing the bubbles from the evaporator.

10. Refrigerating apparatus comprising in combination a closed system including an evaporating element and a condensing element connected thereto and sulphur dioxide and oil capable of forming sustained bubbles in the presence of the refrigerant in the system.

In testimony whereof I hereto affix my signature.

RALPH K. MILLER.

110

115

120

125

130